

## UNITED STATES PATENT OFFICE

2,442,596

## DRY MIXES FOR USE IN ELECTROLYTIC RECORDING

Harold G. Greig, Princeton, N. J., assignor to  
 Radio Corporation of America, a corporation of  
 Delaware

No Drawing. Application November 4, 1944,  
 Serial No. 562,032

17 Claims. (Cl. 204—2)

1

The present invention relates to dry stable mixes for use in preparing solutions for the electrolytic preparation of colored images on a traveling web or band which for simplicity may be referred to as a receiver.

The production of color image records by electrolyzing a solution containing a diazotizable amine, a nitrite, an electrolyte such as sodium chloride, potassium chloride and the like and a coupler, is disclosed in Solomon U. S. P. 2,306,471. In my copending application, Serial No. 562,033, filed of even date herewith and entitled "Electrolytic recording," it is suggested that there be substituted for the amine and nitrite of such solution a stabilized diazo amino compound. Manifold advantages, including an improved stability of the records to light, are obtained when operating in this way. It has been found that these two methods are the most efficacious for electrolytically producing color image records especially in facsimile recording. By the term "facsimile recording" as used herein is meant not only the reproduction on the receiver of a pre-existing subject, but also the reception of subject-matter in the process of creation or formation.

The production from dry mixes of the electrolytic recording solutions with which the receiver is treated in these methods has manifest advantages. If the dry mix be storage stable, it can be prepared in bulk and stored for a considerable period of time. Furthermore, it can be shipped to whatever destination desired at a much lower cost than the water solutions. The production of dry mixes suitable for use in these processes has accordingly been a desiredatum in this art.

The couplers which have been found to give best results in the methods previously outlined are naphthol sulfonic acids, of which chromotropic acid is an example. This acid is usually sold in the form of its mono-sodium salt. This salt is acid and if incorporated into a dry mix containing a diazotizable amine and a nitrite or a stabilized diazo amino compound, it would induce premature diazotization and coupling in the first instance, and premature splitting of the diazo amino compound and coupling in the second instance. If, on the other hand, the alkalinity of such compounds be increased to avoid such premature action by the utilization of the

usual alkalies such as sodium hydroxide, sodium carbonate, potassium hydroxide, and the like, it is found that the records obtained suffer because of a poor shade of the images and because of the instability of the background to light. It has therefore been considered preferable, up to the present time, to prepare fresh solutions for electrolytic recording rather than to produce dry mixes which can be stored and shipped for use at 10 a time in the future despite the advantages inherent in the latter course of action.

I have now discovered that the objections to the dry mixes which has been previously proposed can be avoided by utilizing as the coupling compound in such dry mixes a naphthol sulfonic acid, either mono- or poly-, in which at least one of the sulfonic acid groups is neutralized by morpholine. The morpholine forms a salt of the naphthol sulfonic acids. Such salts are stable 15 and dissolve in water in the concentrations in which they are used in electrolytic recording to give a pH of approximately 9.5. The alkalinity induced by using the morpholine prevails during storage so that no premature diazotization or 20 splitting of the diazo amino compound with resulting coupling takes place. Due to the stability of such salts or to some other as yet unascertained property thereof, solutions in water or another suitable solvent such as alcohol of dry 25 mixes containing said salts, produce on electrolysis, dark image records the background of which has a much higher permanence to light than records obtained where the alkalinity has been produced by resort to the usual alkalies.

It is accordingly an object of my invention to produce dry mixes for the production of electrolytic recording solutions wherein the coupling compound is a naphthol sulfonic acid in which at least one sulfonic acid group has been neutralized by morpholine.

It is a further object of my invention to produce dry mixes for the production of electrolytic recording solutions wherein the coupling compound is a naphthol polysulfonic acid in which at least one sulfonic acid group has been neutralized by morpholine.

It is a further object of my invention to produce storage stable dry mixes containing a primary aromatic amine, a nitrite, an electrolyte 45 and a naphthol sulfonic acid as the coupling com-

pound in which at least one sulfonic acid group has been neutralized with morpholine.

It is a further object of my invention to produce storage stable dry mixes of a stabilized diazo amino compound, an electrolyte and as the coupling compound a naphthol sulfonic acid at least one of the sulfonic acid groups of which has been neutralized with morpholine.

It is a further object of my invention to produce records by electrolyzing a solution containing a 10 source of diazonium ions, an electrolyte, and as a coupling compound a naphthol sulfonic acid in which a sulfonic acid group has been neutralized by morpholine.

It is a further object of my invention to produce dry mixes for forming electrolytic recording solutions in which the coupling compound is chromotropic acid, the sulfonic acid groups of which have been neutralized by morpholine.

It is a further object of my invention to produce dry mixes for electrolytic recording solutions in which the coupling compound is chromotropic acid, the two sulfonic acid groups of which have been neutralized by morpholine.

Further objects of my invention will appear as the description proceeds.

It has been stated that the dry mixes of the present invention contain either a diazotizable amine and a nitrite or a stabilized diazo amino compound. In other words, the diazonium ions which react with the coupling component have their origin in the diazotizable amine and a nitrite on the one hand, or a stable diazo amino compound on the other hand, and accordingly the term "source of diazonium ions" as used in the claims should be so construed. The diazotizable amine or the aryl amine from which the stabilized diazo amino compound is produced may be any of the diazotizable aryl amines utilized in the azo dyestuff art. Examples of such amines are given in the aforesaid Solomon patent and in my copending application, Serial No. 562,033, filed of even date herewith and entitled "Electrolytic recording," to which attention is directed. Such amines are, for example, naphthionic acid, 4,4'-diaminodiphenyl-2,2'-disulfonic acid, 4,4'-diaminodiphenyl 3,3'-disulfonic acid, 4,4'-diaminodiphenylamine-2-sulfonic acid, orthotolidine-2,2'-disulfonic acid, alpha-naphthylamine-4,8-disulfonic acid, alpha-naphthylamine-5-sulfonic acid, o-anisidine-4-sulfonic acid, and the like. These amines when used in the form of the stabilized diazo amino compounds may have their diazonium compounds stabilized with an aliphatic amine such as ethanolamine, diethanolamine, sarcosine, diisopropanolamine, dimethylamine, diethylamine and the like, by an aromatic amine which does not readily couple, such as 4-sulfo-2-aminobenzoic acid, 2-methylamino-4-sulfonylbenzoic acid and the like, or by a heterocyclic amine, such as alpha-carboxy pyrrolidine, alpha-1-alpha-2-dicarboxy pyrrolidine, piperidine, carbazole and the like.

The stabilized diazo amino compounds are prepared by diazotizing the primary aromatic amine and reacting the resulting diazonium compound in an alkaline solution with one of the aforesaid organic amines which does not easily couple to form an azo dye. It is advisable when producing the stabilized compound, to use an excess of the stabilizing amine over the quantity theoretically necessary to produce the stabilized diazonium compound since otherwise difficulties may be encountered in the stability of the records to light.

As the coupling component there may be used any naphthol sulfonic acid at least one sulfo group of which has been neutralized by morpholine. Such compounds have the following formulae:



wherein  $n$  is 1 or 2,  $m$  is 1 to 3 and R is hydrogen or a substituent group, such as, amino, acetyl, amino and the like. As examples of such naphthols, the morpholine salts of which are contemplated by the present invention, may be mentioned.

- 25 2-naphthol-6-sulfonic acid
- 25 2-naphthol-8-sulfonic acid
- 15 1-hydroxy-8-acetylamino naphthalene-3,6-disulfonic acid
- 15 1-hydroxy-8-amino naphthalene-3,5-disulfonic acid
- 30 1-hydroxy-8-amino naphthalene - 6,7-disulfonic acid
- 30 1,8-dihydroxynaphthalene-3,6-disulfonic acid
- 30 1-hydroxy-8-amino naphthalene-3,6-disulfonic acid
- 35 1-hydroxy naphthalene-3,6-disulfonic acid
- 35 2-hydroxy-naphthalene-3,6-disulfonic acid
- 35 1,7-dihydroxy naphthalene-3,6-disulfonic acid
- 35 2-hydroxynaphthalene-6,8-disulfonic acid
- 40 1-hydroxynaphthalene-3,6,8-trisulfonic acid
- 40 1,3-dihydroxynaphthalene-5,7-disulfonic acid
- 40 1,5-dihydroxynaphthalene-2,7-disulfonic acid
- 40 1,5-dihydroxynaphthalene-3,7-disulfonic acid
- 45 1,7-dihydroxynaphthalene-3,6-disulfonic acid
- 45 1 - hydroxy-7-amino naphthalene-3,6-disulfonic acid

and the like. Best results, however, have been secured with the salts of chromotropic acid and the use of the salt of this acid represents the preferred embodiment of my invention.

The preparation of the morpholine derivative of the coupling compound may be carried out in various ways. For instance, if the morpholine salt—say, of chromotropic acid—is desired, 1 mol of the mono-sodium salt of chromotropic acid is slurried with sufficient morpholine in excess of 2 mols to give a smooth, uniformly wet paste. The excess morpholine is then removed by drying at a temperature of about 65 to 70° C. As an alternative, 1 mol of chromotropic acid itself is reacted with 2 mols of morpholine at room temperature in a closed vessel, for instance, a ball mill, by means of which thorough mixing of the reactants can be accomplished. The morpholine is sufficiently volatile so that any excess over that which combines with the coupling agent is readily driven off at the temperatures of 65 to 70° C. referred to above.

It has been previously pointed out that at 70 least one of the sulfonic acid groups of the coupling component is neutralized by morpholine. If the naphthol sulfonic acid employed is a mono-sulfonic acid, only the monoamine salt is formed, in which case the preparation is effected by 75 using 1 mol of the naphthol sulfonic acid with

at least 1 mol of morpholine. Where the coupling component is a polysulfonic acid, the ratio of the reactants will vary depending upon the particular naphthol polysulfonic acid selected and the results desired. If, for instance, a disulfonic acid such as chromotropic acid is used, a monoamine salt may be prepared by using 1 mol of the sulfonic acid for each mol of morpholine. If, however, the di-salt is desired, at least 2 mols of morpholine are used for each mol of the chromotropic acid. Thus the gain in weight when slurrying the monosodium salt of chromotropic acid with a large excess of morpholine and drying, leads to a product containing 2 mols of morpholine and 1 mol of chromotropic acid. Similarly, if the polysulfonic acid is a trisulfonic acid, by adjusting the proportions in the manner noted, the mono-, di- or triamine salt may be produced.

It is also possible to produce salts of the naphthol polysulfonic acids in which one sulfonic acid group is neutralized with morpholine and another group is neutralized by means of an alkali metal. It is thus possible when starting with 1 mol of the mono-sodium salt of chromotropic acid and treating the same with 1 mol of morpholine to obtain a mixed sodium-morpholine salt. Again, by operating as indicated above, that is, by using a naphthalene disulfonic acid such as chromotropic acid, with 1 mol of an alkyloamine and 1 mol of morpholine, it is possible to prepare the mixed alkyloamine-morpholine salt.

The dry mixture which is used, irrespective of the source of the diazonium compound, must contain an electrolyte. The electrolyte is preferably sodium chloride, although other common electrolytes such as potassium chloride, sodium bromide and the like may be utilized with equally good results.

The preferred pH of the solution resulting from dissolving the dry mixture in water is between 9.5 and 11.5. In some instances, the alkalinity afforded by the salt of the coupling agent will not give the pH which is optimum for the component used. In that case, it is desirable to add a very small amount of an inorganic alkali such as sodium hydroxide, potassium hydroxide or the like. The quantity of this agent required will usually be from 1 to 2 grams per liter of the recording solution.

Other ingredients may be incorporated in the dry mix and in particular a wetting agent to facilitate the impregnation of the carrier by the solution. Suitable wetting agents are sarcosines or taurines, the nitrogen atom of which is acylated with a high molecular weight fatty acid such as oleic, palmitic, or the like, alkyl naphthalene sulfonic acids, such as butyl naphthalene sulfonate, and the like, and the condensation product of a sulfonated benzene with chlorinated kerosene, said condensation product having the formula:



wherein R represents the hydrocarbon radicals present in kerosene (see U. S. P. 2,220,099). The wetting agent will usually be present in an amount ranging from .05 to about 1 gram per liter of solution.

The invention will be further understood from the following examples, but it is to be remem-

bered that these examples are illustrative and not limitative.

#### Example I

5 .2 gram-mol of the mono-sodium salt of chromotropic acid in the form of a finely ground dry powder is slurried with 1.1 gram-mols of morpholine until a smooth, thick paste is obtained. This paste is stirred at room temperature until 10 the mass has become uniform and thoroughly wet throughout. The excess morpholine is then driven off by heating the composition to a temperature of 65-70° C. The product thus obtained is then ground for further use. When 15 dissolved in water in the ratio of .03 gram-mol per liter, it gives a solution of a pH of about 9.5.

.2 gram mol of said morpholine salt of chromotropic acid, .4 gram mol of the diazo compound from diazotized naphthionic acid and diethanolamine, 3.3 grams of the condensation 20 product of benzene sulfonic acid with chlorinated kerosene, 163.8 grams of sodium chloride, and 8.2 grams of sodium hydroxide are thoroughly ground and mixed together to produce a uniform dry product.

25 74.5 grams of this mixture are dissolved in a liter of water for the preparation of a facsimile recording solution. This solution has a pH of 10.1. Records produced with such a solution 30 are a dark blue purple, the background of which has a high stability to light.

The diazo amino compound from diazotized naphthionic acid and diethanolamine referred to above is obtained as follows:

35 .5 gram mol of sodium naphthionate are dissolved in approximately 750 cc. of water to which sufficient sodium hydroxide is added to make the solution alkaline to brilliant yellow test paper.

40 5 gram mol of sodium nitrite is then added and the solution is run under rapid agitation at a temperature of 5 to 10° C. into a solution of 140 cc. of 38% hydrochloric acid and 750 cc. of water and ice. Diazotization is complete almost 45 as soon as the solution is added and the diazonium compound, which is quite insoluble, precipitates out as a thick, creamy slurry. Stirring is continued for one hour to obtain the product in a form in which it is more easily filtered.

50 The filter cake obtained upon filtration is re-slurried in approximately 500 cc. of water until a smooth paste is obtained. This paste is added slowly at 10 to 15° C. over a two-hour period with rapid agitation to a solution of 125 cc. of 55 diethanolamine in 250 cc. of water while maintaining a temperature of 10 to 15° C. in an ice bath to minimize decomposition.

The reaction is complete when all the diazonium compound has been added. The resulting 60 solution is amber in color and may stain paper with a reddish tint. It must be alkaline when tested with brilliant yellow test solution.

2 grams of sodium hydrosulfite are added and the solution stirred for one hour at room temperature to clear away the red-staining impurities. 20 grams of activated charcoal are incorporated and the temperature raised to 50 to 55° C. for 1/2 hour for the purpose of further clarifying the solution and to remove basic impurities. The solution is then filtered and the volume is adjusted to 1000 cc.

#### Example II

.075 gram mol of diisopropanolamine are dissolved in .574 gram mol of morpholine. .10 gram

mol of chromotropic acid in a dry, finely ground condition are slurried with the morpholine solution. The product is then treated at a temperature of about 70° C. A product having a dry weight of 74.04 grams and dark gray in color is thus obtained. The product appears to be a mixed salt of diisopropanolamine and morpholine. When substituted for the chromotropic acid-morpholine salt of Example I and the mix used in electrolytic recording, blue-purple records are obtained.

*Example III*

The procedure is the same as in Example I except that the chromotropic acid is replaced by 1 - hydroxy-8-amino-naphthalene-6,7-disulfonic acid.

*Example IV*

The procedure is the same as in Example I except that the chromotropic acid is replaced by 2-hydroxy-naphthalene-3,6-disulfonic acid.

*Example V*

The procedure is the same as in Example I except that the chromotropic acid is replaced by 1,7-dihydroxynaphthalene-3,6-disulfonic acid.

*Example VI*

.03 gram mol of sodium naphthionate, .02 gram mol of sodium nitrite, 1. gram mol of sodium chloride, and .015 gram mol of the chromotropic acid-morpholine salt of Example I are thoroughly ground and mixed together to produce a uniform product. To the mixture there is added a small amount of sodium hydroxide approximating 1 gram.

The above dry mixture is stable and will remain so for a prolonged period of time. A receiver treated with a water solution of the same and subjected to the action of an electrolytic current gives purple-blue records having a background stable to light.

*Example VII*

The procedure is the same as in Example VI except that for the sodium naphthionate there are used .06 gram mol of 4,4'-diamino-diphenyl-3,3'-disulfonic acid and .5 gram mol of sodium nitrite.

*Example VIII*

.02 gram mol of chromotropic acid is ground in a ball mill with .02 gram mol of morpholine. The resulting product is dried at a temperature of about 65° C. The product, which is the mono-morpholinium salt of chromotropic acid, may be substituted for the di-salt of Example I.

*Example IX*

.02 gram mol of 1-hydroxy-naphthalene-3,6-disulfonic acid and .02 gram mol of morpholine are treated in a ball mill to effect a thorough mixing of the reagents. The product when dried at a temperature of 70° C. may be used in lieu of the morpholine treated salt of Example I. Said product is the mono-morpholinium salt of 1-hydroxy-naphthalene-3,6-disulfonic acid.

The carrier which is treated with a solution of the above dry mixes may be paper, a fabric or the like. During electrolysis, dyestuff formation occurs only at the anode, which means that the image record appears on only one surface of the receiver. The image will of course vary in intensity, depending upon the impulses which are applied to the electrodes.

Various modifications of the invention will occur to persons skilled in the art and I therefore do not intend to be limited in the patent granted except as required by the prior art and the appended claims.

I claim:

1. A storage-stable dry mix for use in producing electrolytic recording solutions containing as its essential components a source of diazonium ions capable of yielding a diazonium compound under the influence of an electrolytic recording current, a water soluble inorganic salt as the electrolyte in an amount to insure passage of the electrolytic recording current through such solution, a sufficient quantity of a naphthol sulfonic acid, a sulfonic acid group of which has been neutralized by morpholine to couple with the diazonium compound when formed to produce an azo dye, said composition when dissolved in water having a pH on the alkaline side.

2. A storage-stable dry mix for use in producing electrolytic recording solutions comprising as its essential components a diazotizable amine, a sufficient quantity of an ionizable nitrite to produce the nitrite ions necessary for diazotization of said amine under the influence of an electrolytic recording current, a water soluble inorganic salt as an electrolyte in an amount to insure passage of the electrolytic recording current, and a sufficient quantity of a naphthol sulfonic acid in which at least one of the sulfonic acid groups is neutralized by morpholine to couple with the diazonium compound when formed to produce an azo dye, said composition when dissolved in water having a pH on the alkaline side.

3. A storage-stable dry mix for producing electrolytic recording solutions containing as its essential components a diazo amino compound capable of yielding a diazonium compound under the influence of an electrolytic recording current, a water soluble inorganic salt as the electrolyte in an amount to insure passage of the electrolytic recording current and a sufficient quantity of a naphthol sulfonic acid in which at least one sulfonic acid group is neutralized by morpholine to couple with the diazonium compound when formed to produce an azo dye, said composition when dissolved in water having a pH on the alkaline side.

4. A storage-stable dry mix for producing electrolytic recording solutions containing as its essential components a source of diazonium ions capable of yielding a diazonium compound under the influence of an electrolytic recording current, a water soluble inorganic salt as the electrolyte in an amount to insure passage of the electrolytic recording current, and a sufficient quantity of a naphthol polysulfonic acid at least one sulfonic acid group of which is neutralized by morpholine to couple with said diazonium compound when formed to produce an azo dye, said composition when dissolved in water having a pH on the alkaline side.

5. A storage-stable dry mix for producing electrolytic recording solutions containing as its essential components a diazotizable amine, a sufficient quantity of an ionizable nitrite to produce the nitrite ions necessary to diazotize said amine under the influence of the electrolytic recording current, a water soluble inorganic salt as the electrolyte in an amount to insure passage of the electrolytic recording current and a sufficient quantity of a naphthol polysulfonic acid in which at least one of the sulfonic acid groups is neutralized by morpholine to couple with the diazonium com-

pound when formed to produce an azo dye, said composition when dissolved in water having a pH on the alkaline side.

6. A storage-stable dry mix for producing electrolytic recording solutions containing as its essential components a diazo amino compound capable of yielding a diazonium compound under the influence of an electrolytic recording current, a water soluble inorganic salt as the electrolyte in an amount to insure passage of the electrolytic recording current, and a sufficient quantity of a naphthol polysulfonic acid in which at least one sulfonic acid group is neutralized by morpholine to couple with said diazonium compound when formed to produce an azo dye, said composition when dissolved in water having a pH on the alkaline side.

7. A storage-stable dry mix for producing electrolytic recording solutions containing as its essential components, sodium naphthionate, a sufficient quantity of sodium nitrite to produce the nitrite ions necessary for diazotization of said sodium naphthionate under the influence of an electrolytic recording current, a water soluble inorganic alkali metal salt as the electrolyte in an amount to insure passage of the electrolytic recording current and a sufficient quantity of a morpholinium salt of chromotropic acid to couple with the diazonium compound when formed to produce an azo dye, said composition when dissolved in water having a pH on the alkaline side.

8. A storage-stable dry mix for producing electrolytic recording solutions containing as its essential components the diazo amino compound of diazotized naphthionic acid and diethanolamine capable of yielding a diazonium compound under the influence of an electrolytic recording current, a water soluble inorganic salt as the electrolyte in an amount to insure passage of the electrolytic recording current, and a sufficient quantity of a morpholinium salt of chromotropic acid to couple with the diazonium compound when formed to produce an azo dye, said composition when dissolved in water having a pH on the alkaline side.

9. The composition as defined in claim 5 wherein the morpholine salt is the di-salt of chromotropic acid.

10. The process of producing color images on a moving fibrous receiver by the electrolytic facsimile recording method which comprises impregnating the receiver with an alkaline solution of a source of diazonium ions capable of yielding a diazonium compound under the influence of the

electrolytic recording current, a water soluble inorganic salt as the electrolyte in an amount to insure passage of the electrolytic recording current and a sufficient quantity of a naphthol sulfonic acid at least one sulfonic acid group of which is neutralized by morpholine to couple with the diazonium compound when formed to produce an azo dye and subjecting the so treated receiver to the action of an electrolytic recording current.

10 11. The process as defined in claim 10 wherein said source of diazonium ions is a diazotizable amine and a nitrite.

15 12. The process of producing color images on a moving fibrous receiver by the electrolytic facsimile recording method which comprises impregnating the receiver with an alkaline solution of diazotized naphthionic acid stabilized with diethanolamine, capable of yielding a diazonium compound under the influence of an electrolytic recording current, sodium chloride as the electrolyte in an amount to insure passage of the electrolytic recording current and a sufficient quantity of a morpholinium salt of chromotropic acid to couple with the diazonium compound when formed to produce an azo dye and subjecting the so treated receiver to the action of an electrolytic recording current.

20 13. A fibrous sheet material impregnated with an aqueous solution of the composition of claim 1.

25 14. A fibrous sheet material impregnated with an aqueous solution of the composition of claim 2.

15 15. A fibrous sheet material impregnated with an aqueous solution of the composition of claim 3.

20 16. A fibrous sheet material impregnated with an aqueous solution of the composition of claim 7.

25 17. A fibrous sheet material impregnated with an aqueous solution of the composition of claim 8.

40 HAROLD G. GREIG.

#### REFERENCES CITED

The following references are of record in the file of this patent:

#### 45 UNITED STATES PATENTS

| Number    | Name    | Date          |
|-----------|---------|---------------|
| 2,135,964 | Dahlen  | Nov. 28, 1938 |
| 2,306,471 | Solomon | Dec. 29, 1942 |

#### 50 OTHER REFERENCES

The Aromatic Diazo-Compounds and Their Technical Applications, by K. H. Saunders, published by Edward Arnold and Co., London 1936, pages 108, 109, 110.